

# United States Patent [19]

van Konyenborg et al.

[11] Patent Number: 4,935,156

[45] Date of Patent: Jun. 19, 1990

## [54] CONDUCTIVE POLYMER COMPOSITIONS

[75] Inventors: Peter H. van Konyenborg, Palo Alto; Andrew Au, Fremont, both of Calif.

[73] Assignee: Raychem Corporation, Menlo Park, Calif.

[21] Appl. No.: 423,589

[22] Filed: Sep. 27, 1982

### Related U.S. Application Data

[63] Continuation-in-part of Ser. No. 300,709, Sep. 9, 1981, abandoned.

[51] Int. Cl.<sup>5</sup> ..... H01B 1/06

[52] U.S. Cl. ..... 219/553; 252/511; 338/22SD; 338/22 R

[58] Field of Search ..... 219/528, 549, 553, 548; 338/22 R, 22SD; 524/545, 495, 496, 300, 709; 252/511

## [56] References Cited

### U.S. PATENT DOCUMENTS

- 2,978,665 7/1956 Vernet et al. ..... 338/223  
3,823,217 7/1974 Kampe ..... 264/105  
3,935,159 1/1976 Demillecamp et al. ..... 524/545 X  
4,237,441 12/1980 van Konyenborg et al. .... 252/511 X  
4,251,432 2/1981 Martin ..... 524/545 X  
4,304,987 12/1981 Konyenborg ..... 252/511  
4,328,151 5/1982 Robinson ..... 524/545 X

## FOREIGN PATENT DOCUMENTS

- 1805906 6/1969 Fed. Rep. of Germany .  
1373711 11/1974 United Kingdom .  
1449261 9/1976 United Kingdom .  
1469311 4/1977 United Kingdom .  
1469312 4/1977 United Kingdom .  
2075992A 11/1981 United Kingdom .

## OTHER PUBLICATIONS

European Search Report, 12/22/82.

U.K. Search Report, 10/19/82.

Primary Examiner—Josephine Barr

Attorney, Agent, or Firm—Timothy H. P. Richardson; Herbert G. Burkard

[57]

### ABSTRACT

Conductive polymer compositions based on polyvinylidene fluoride have improved properties when the polyvinylidene fluoride has a very regular structure which can be characterized by a low head-to-head content in the repeating units. The improved properties include electrical stability when contacted by organic fluids and/or when maintained at elevated temperatures in air. Such compositions which exhibit PTC behavior are particularly useful in the form of self-limiting heaters which are immersed in organic fluids, especially flexible strip heaters for heating diesel fuel before it passes through a fuel filter.

16 Claims, 2 Drawing Sheets





FIG\_1



FIG\_2

## CONDUCTIVE POLYMER COMPOSITIONS

## CROSS-REFERENCE TO RELATED APPLICATION

This application is a continuation-in-part of our pending application Ser. No. 300,709 filed Sept. 9, 1981, now abandoned, the entire disclosure of which is incorporated herein by reference.

## BACKGROUND OF THE INVENTION

## 1. Field of the Invention

This invention relates to conductive polymer PTC compositions and devices comprising them.

## 2. Introduction to the Invention

Conductive polymer compositions, and devices comprising them, are known. Reference may be made for example to U.S. Pat. Nos. 2,978,665, 3,243,753, 3,351,882, 3,571,777, 3,793,716, 3,823,217, 3,861,029, 4,017,715, 4,177,376, 4,188,276, 4,237,441, 4,238,812, 4,242,573, 4,246,468, 4,255,698, 4,388,607, 4,426,339, 4,538,889 and 4,560,498; U.K. Patent No. 1,534,715; the article entitled "Investigations of Current Interruption by Metal-filled Epoxy Resin" by Littlewood and Briggs in J. Phys D: Appl. Phys, Vol. II, pages 1457-1462; the article entitled "The PTC Resistor" by R. F. Blaha in Proceedings of the Electronic Components Conference, 1971; the report entitled "Solid State Bistable Power Switch Study" by H. Shulman and John Bartho (August 1968) under Contract NAS-12-647, published by the National Aeronautics and Space Administration; J. Applied Polymer Science 19, 813-815 (1975), Klason and Kubat; Polymer Engineering and Science 18, 649-653 (1978) Narkis et al; and commonly assigned U.S. Ser. Nos. 601,424 (Moyer), now abandoned, published as German OLS 2,634,999. For details of more recent developments in this field, reference may be made to copending and commonly assigned U.S. Ser. Nos. 67,207 (Doljack et al.) now abandoned in favor of continuation-in-part application Ser. No. 228,347, now Patent No. 4,450,496, 98,711 (Middleman et al.), now Patent No. 4,315,237, 141,984 (Gotcher et al.), 141,987 (Middleman et al.), now Patent No. 4,413,301 141,988 (Fouts et al.), 141,989 (Evans), 141,991 (Fouts et al.), 142,053 (Middleman et al.), now Patent No. 4,352,083, 142,054 (Middleman et al.), now Patent No. 4,317,027, 150,910 (Sopory), now Patent No. 4,334,351, 150,911 (Sopory), now Patent No. 4,318,881, 174,136 (Cardinal et al.), now Patent No. 4,314,230, 176,300 (Jensen), now Patent No. 4,330,704, 250,491 (Jacobs et al.), 254,352 (Taylor), now Patent No. 4,426,633, 272,854 (Stewart et al.), now abandoned in favor of continuation-in-part application Ser. No. 403,203, now Patent No. 4,502,929, 273,525 (Walty) now Patent No. 4,398,084 and 274,010 (Walty et al.), now abandoned. The disclosure of each of the patents, publications and applications referred to above is incorporated herein by reference.

Electrical devices containing conductive polymers generally (though not invariably) comprise an outer jacket, usually of insulating material, to protect the conductive polymer from damage by the surrounding environment. However, if no protective jacket is used, or if the jacket is permeable to harmful species in the environment, or if the conditions of use are such that the jacket may become damaged, it is necessary or desirable to select a conductive polymer which is not damaged (or which deteriorates at an acceptably low rate) when exposed to the surrounding environment. Exposure of

conductive polymers to organic fluids generally results in an increase in resistivity; exposure to air, especially at elevated temperatures between room temperature and 35° C. below the melting point generally results in a decrease in resistivity both at the elevated temperature and at room temperature (a phenomenon known in the art as "resistance relaxation").

## SUMMARY OF THE INVENTION

10 We have discovered that conductive polymer compositions which are based on polyvinylidene fluoride exhibit substantially improved stability if the polyvinylidene fluoride has a very regular structure which can be characterized by a low head-to-head content in the repeating units. Polyvinylidene fluoride is made up of repeating units of formula  $-\text{CH}_2\text{CF}_2-$ , which can be arranged head-to-tail (i.e.  $-\text{CH}_2\text{CF}_2-\text{CH}_2\text{CF}_2-$ ) or heat-to-head (i.e.  $-\text{CH}_2\text{CF}_2-\text{CF}_2\text{CH}_2-$ ), and we have found that the lower the heat-to-head content, the greater the stability of the resistivity of the composition when exposed to organic fluids and/or when exposed to air at elevated temperature. Previously known conductive polymer compositions based on polyvinylidene fluoride have made use of polyvinylidene fluoride of relatively high head-to-head content, namely at least 5.2% and generally higher, which are easier to process than the polymers used in the present invention.

15 In its first aspect, the present invention provides a conductive polymer composition which comprises (a) polyvinylidene fluoride having a head-to-head content of less than 5.0%, preferably less than 4.5%, particularly less than 4.0%, and (b) a particulate conductive filler, especially carbon black, dispersed in the polyvinylidene fluoride. The composition preferably exhibits PTC behavior.

20 In its second aspect, the invention provides an electrical device which comprises a conductive polymer element composed of a conductive polymer composition as defined above and at least one electrode in electrical contact with said element, for example, at least two electrodes which can be connected to a source of electrical power and which when so connected cause current to flow through the conductive polymer element.

## BRIEF DESCRIPTION OF THE DRAWING

The invention is illustrated in the accompanying drawing, in which FIGS. 1 and 2 show the effect on resistivity of immersing two conductive polymer compositions in various organic solvents.

## DETAILED DESCRIPTION OF THE INVENTION

25 Polyvinylidene fluorides suitable for use in this invention are commercially available. The head-to-head content of a polyvinylidene fluoride can be measured by those skilled in the art. We have found that the measured heat-to-head contents of different samples of a polymer sold under a particular trade name can differ substantially. In general, the presently available polyvinylidene fluorides made by suspension polymerization (rather than emulsion polymerization) have lower head-to-head contents. The number average molecular weight of the polymer is generally at least 5,000, e.g. 7,000 to 15,000.

30 The polyvinylidene fluoride is preferably a homopolymer of vinylidene fluoride, but the presence of small quantities of comonomers, (preferably less than 15%,

particularly less than 5% by weight), eg. tetrafluoroethylene, hexafluoropropylene and ethylene, is not excluded. The polyvinylidene fluoride is preferably the sole crystalline polymer in the composition, but other crystalline polymers, eg. other crystalline fluoropolymers, may also be present. The composition may contain relatively small amounts (preferably less than 35%, especially less than 20%, particularly less than 10%, by volume) of one or more elastomeric polymers, particularly solvent-resistant fluorine-containing elastomers and acrylic elastomers, which are usually added primarily to improve the flexibility and elongation of the composition.

The particulate conductive filler preferably comprises carbon black, and often consists essentially of carbon black. Choice of the carbon black will influence the resistivity/temperature characteristics of the composition. Compositions exhibiting PTC behavior are preferred for many devices of the invention, especially self-limiting heaters, and for these a carbon black having a ratio of surface area ( $m^2/g$ ) to particle size ( $\mu$ ) of 0.03 to 6.0 is preferred. For other uses, compositions exhibiting ZTC or NTC behavior may be preferred. The amount of conductive filler used will depend upon the desired resistivity of the composition. For flexible strip heaters which are to be used for heating diesel fuel and powered by a 12 volt battery, we prefer a PTC

comparative Examples not in accordance with the invention.

#### EXAMPLE 1

The ingredients listed for Composition A in Table 1 below were mixed in a Banbury mixer. The mixture was dumped, placed on a steam-heated mill and extruded into a water bath through a 3.5 inch (8.9 cm) extruder fitted with a pelletizing die. The extrudate was chopped into pellets which are dried for 16 hours at 80° C.

The ingredients listed for Composition B in Table 1 were mixed and pelletized in the same way as for Composition A.

83% by weight of the Composition A pellets and 17% by weight of the Composition B pellets were tumble blended and dried at 110° C. The composition of the resulting Final Blend is shown in Table 1. Using a 1.5 inch (3.8 cm) diameter extruder fitted with a crosshead die having an orifice 0.4 inch (1.0 cm)  $\times$  0.1 inch (0.3 cm), the blend was melt-extruded over a pair of pre-heated 14 AWG (1.85 mm diameter) 19/27 nickel-coated copper wires with a center-to-center separation of 0.25 inch (0.64 cm). The extrudate was passed immediately through a bath of water at room temperature, air-dried, and then irradiated to a dosage of 10 Mrad. The conductive polymer had a resistivity of about 50 ohm.cm at 25° C.

TABLE 1

|             | Composition B |      |       | Composition A |      |       | Final Blend |       |
|-------------|---------------|------|-------|---------------|------|-------|-------------|-------|
|             | Wt (g)        | Wt % | Vol % | Wt (g)        | Wt % | Vol % | Wt %        | Vol % |
| Kynar 460   | 16,798        | 72   | 72.6  | 16,339        | 70   | 70.6  | 71.7        | 72.3  |
| Furnex N765 | 4,433         | 19   | 18.7  | 4,901         | 21   | 20.7  | 19.3        | 19.0  |
| Viton AHV   | 1,400         | 6    | 5.9   | 1,400         | 6    | 5.9   | 6.0         | 5.9   |
| Omya-BSH    | 467           | 2    | 1.3   | 467           | 2    | 1.3   | 2.0         | 1.3   |
| TAIC        | 233           | 1    | 1.5   | 233           | 1    | 1.5   | 1.0         | 1.5   |

Kynar 460 is polyvinylidene fluoride available from Pennwalt and having a head-to-head content of about 5.5%.

Furnex N765 is a carbon black available from Columbia Chemical having a particle size of about 60 millimicrons, a surface area of about 32  $m^2/g$  and a DBP value of about 112  $cm^3/100\text{ g}$ .

Viton AHV is a copolymer of hexafluoropropylene and polyvinylidene fluoride manufactured by du Pont.

Omya-BSH is calcium carbonate available from Omya Inc.

TAIC is triallyl isocyanurate, a radiation cross-linking agent.

composition whose resistivity at 25° C. is less than 200 ohm.cm eg. about 10 to about 100 ohm.cm. In such compositions the amount of carbon black may for example be 16 to 25% by weight.

In addition to one or more conductive fillers, the compositions may also comprise other conventional additives, such as non-conductive fillers (including flame retardants), antioxidants and crosslinking agents (or residues thereof if the composition has been cross-linked).

The compositions of the invention are preferably cross-linked (particularly by irradiation), since this has been found to enhance their resistance to organic solvents.

Preparation of the compositions of the invention can be carried out in conventional fashion. Often it will be convenient to melt-extrude the composition directly into a water bath (which may be heated), and using this technique subsequent annealing is often not required.

The invention is illustrated by the following Examples, in which Examples 1, 2, 3, 7, 12 and 13 are Com-

#### EXAMPLES 2-6

The ingredients listed for Examples 2 to 6 in Table 2 below were mixed in a Banbury mixer. The mixture was dumped, granulated and dried for 72 hours at 75° C. under vacuum. Using a 0.75 inch (1.9 cm) single screw extruder fitted with a cross-head die having an orifice 0.3 inch (0.76 cm)  $\times$  0.1 inch (0.3 cm), the blend was melt-extruded over a pair of pre-heated 18 AWG (1.2 mm diameter) 19/27 nickel-coated copper wires with a center-to-center separation of 0.25 inch (0.64 cm). The extrudate was passed immediately through a bath of water at room temperature, air-dried, and then irradiated to a dosage of 10 Mrad.

#### EXAMPLES 7-15

The ingredients shown for Examples 7-15 in Table 2 were mixed in a Banbury mixer, dumped and then granulated. The granulated materials were molded into slabs of thicknesses of 0.030" (0.076 cm) to 0.036" (0.091 cm) by compression molding at 200° C. for three minutes.

TABLE 2

| Ingredients | Ex. No. |    |   |   |   |    |   |   |    |    |     |     |    |
|-------------|---------|----|---|---|---|----|---|---|----|----|-----|-----|----|
|             | 2C      | 3C | 4 | 5 | 6 | 7C | 8 | 9 | 10 | 11 | 12C | 13C | 14 |
| Kynar 450   | 77      |    |   |   |   | 90 |   |   |    |    | 88  |     |    |
| Kynar 460   |         | 77 |   |   |   |    |   |   |    |    | 89  |     |    |

TABLE 2-continued

| Ingredients                          | Ex. No. |    |    |    |    |                   |                   |      |      |      |     |     |      |      |
|--------------------------------------|---------|----|----|----|----|-------------------|-------------------|------|------|------|-----|-----|------|------|
|                                      | 2C      | 3C | 4  | 5  | 6  | 7C                | 8                 | 9    | 10   | 11   | 12C | 13C | 14   | 15   |
| Solef 1010                           |         |    | 74 |    |    |                   | 88.5              | 88   |      |      |     |     |      |      |
| KF1100                               |         |    |    | 74 |    |                   |                   |      | 89.5 |      |     |     |      | 88.5 |
| KF1000                               |         |    |    |    | 77 |                   |                   |      |      |      |     |     |      |      |
| Dyflor 2000 M                        |         |    |    |    |    |                   |                   |      | 89.5 |      |     |     | 88.5 |      |
| Statex G                             | 21      | 21 | 24 | 24 | 21 |                   |                   |      |      |      |     |     |      |      |
| Vulcan XC72                          |         |    |    |    |    | 8                 | 9.5               | 10   | 8.5  | 8.5  | 10  | 9   | 9.5  | 9.5  |
| Omya BSH                             | 2       | 2  | 2  | 2  | 2  | 2                 | 2                 | 2    | 2    | 2    | 2   | 2   | 2    | 2    |
| Resistivity<br>(ohm-cm)<br>at 25° C. |         |    |    |    |    | $3.1 \times 10^4$ | $1.6 \times 10^4$ | 1800 | 1850 | 2000 | 288 | 298 | 200  | 134  |

Kynar 450 is polyvinylidene fluoride available from Pennwalt and having a head-to-head content in the range 5.5 to 6.3.

Solef 1010 is a polyvinylidene fluoride available from Solvay et cie of Belgium, and having a head-to-head content of 4.1%.

KF1000 and KF1100 are polyvinylidene fluorides available from Kureha Chemical Industry Co. of Japan, and having a head-to-head content of 3.5 to 3.8%.

Statex G is a carbon black available from Cities Services Co., Columbian Division having a particle size of about 60 millimicrons, a surface area of about  $32 \text{ m}^2/\text{g}$  and a DBP value of about  $90 \text{ cm}^3/100 \text{ g}$ .

Dyflor 2000 M is a polyvinylidene fluoride available from Kay-Fries, Inc., member of Dynamit Nobel Chemikalien of Federal Republic of Germany and having a head-to-head content of about 4.4-4.9.

Vulcan XC-72 is a carbon black available from Cabot Co., having a particle size of about 30 millimicrons, a surface area of about  $224 \text{ m}^2/\text{g}$  and a DBP value of about  $178 \text{ cm}^3/100 \text{ g}$ .

### TESTS FOR STABILITY IN ORGANIC SOLVENTS

The extrudates obtained in Examples 1 and 4 were compared by the following tests. Samples 2 inch (5.1 cm) long were cut from the extrudates. The samples were immersed in various solvents at 25° C. and the resistance of the samples was measured at intervals. The solvents used, and their solubility parameters, were

| Solvent                   | Solubility Parameter<br>(cal/cm <sup>3</sup> ) <sup>0.5</sup> |
|---------------------------|---------------------------------------------------------------|
| Toluene                   | 8.9                                                           |
| Methylethylketone (MEK)   | 9.3                                                           |
| Acetone                   | 9.9                                                           |
| o - dichlorobenzene       | 10.0                                                          |
| Acetic Anhydride          | 10.3                                                          |
| Pyridine                  | 10.7                                                          |
| Dimethylacetamide (DMAC)  | 10.8                                                          |
| Dimethylsulphoxide (DMSO) | 12.0                                                          |
| Dimethylformamide (DMF)   | 12.1                                                          |
| Ethanol                   | 12.7                                                          |

The results for Examples 1 and 4 are shown in FIGS. 1 and 2 respectively of the accompanying drawings, where the ratio of the resistance at a given time ( $R_t$ ) to the initial resistance ( $R_i$ ) is plotted against time. The greater stability of the composition of the invention (Example 4, shown in FIG. 2) is apparent.

The extrudates obtained in Examples 1 to 6 were compared in the following way. Samples 2 inch (5.1 cm) long were cut from the extrudates and were immersed in various test liquids maintained at 160° F. (71° C.). The test liquids are listed below and include diesel fuel and various commercially available additives for diesel fuel along and mixed with diesel fuel. At intervals, the samples were removed, cooled to 25° C. and dried, and their resistance measured. Table 3 shows the value of the ratio  $R_t/R_i$  for the different samples at various times. The additives tested, and their main ingredients, were as follows:

B12 Toluene, methanol, acetone, naphthalenic mineral oil and ethylene glycol monobutylether.

Fire Prep 100 Naphthalenic oil and partly oxidised aliphatic hydrocarbon

Sta-Lube Naphthalenic mineral oil

Redline and Catalyst Naphthalenic mineral oil, barium carbonate other inorganic carbonates, and sulfur-containing material

Wynn's Conditioner Naphthalenic mineral oil and isopropanol

Gumout Naphthalenic mineral oil, non-aromatic ester and aliphatic acid.

Wynn's Anti-Knock Naphthalenic mineral oil, non-aromatic ester, aliphatic amide, and aliphatic acid.

FPPF Ethyl cellulose, ethylene glycol monobutylether, and oxidised hydrocarbons.

| Example No.                     | 1C(C)            | 2(C)             | 3(C)             | 4                 | 5    | 6    |
|---------------------------------|------------------|------------------|------------------|-------------------|------|------|
| $R_i$ (ohms)                    | 9.3              | 8.8              | 2.3              | 14.1              | 19.7 | 10.4 |
| $R_t/R_i$ after<br>19 hours in  |                  |                  |                  |                   |      |      |
| B12                             | $23 \times 10^4$ | $28 \times 10^4$ | $43 \times 10^4$ | $3.3 \times 10^4$ | 133  | 339  |
| Fire Prep 1000                  | 1.02             | 1.04             | 0.96             | 0.91              | 0.94 | 0.92 |
| Sta-Lube                        | 1.09             | 1.04             | 1.11             | 0.94              | 0.95 | 0.91 |
| Red-line Catalyst               | 1.22             | 1.06             | 1.33             | 1.00              | 0.97 | 1.05 |
| Wynn's Conditioner              | 1.39             | 1.18             | 1.19             | 1.13              | 1.08 | 1.15 |
| Gumout                          | 1.14             | 1.10             | 1.22             | 1.01              | 1.01 | 1.08 |
| Wynn's Anti                     | 1.12             | 1.04             | 1.18             | 0.99              | 1.00 | 1.09 |
| $R_t/R_i$ after<br>110 hours in | 1.03             | 0.97             | 1.07             | 0.93              | 1.00 | 0.92 |
| Diesel Fuel                     |                  |                  |                  |                   |      |      |
| $R_t/R_i$ after 69<br>hours in  |                  |                  |                  |                   |      |      |
| Diesel Fuel +<br>7% B12         | 1.26             | 1.10             | 1.67             | 1.15              | 1.05 | 1.12 |
| Diesel Fuel +<br>7% FPPF        | 1.32             | 1.12             | 1.20             | 1.08              | 1.05 | 1.12 |

-continued

| Example No.                                                                | 1C(C) | 2(C) | 3(C) | 4    | 5    | 6    |
|----------------------------------------------------------------------------|-------|------|------|------|------|------|
| Diesel Fuel + 10% gasoline R/R <sub>0</sub> after 275 hours in Diesel Fuel | 1.17  | 1.05 | 1.15 | 1.01 | 0.99 | 1.07 |
| R/R <sub>0</sub> after 157 hours in Diesel fuel + 7% B12                   | 1.09  | 1.01 | 1.12 | 0.95 | 0.93 | 1.04 |
| Diesel Fuel + 7% FPPF                                                      | 1.78  | 1.30 | 1.47 | 1.17 | 1.14 | 1.27 |
| Diesel Fuel + 10% gasoline                                                 | 1.33  | 1.10 | 1.28 | 1.06 | 1.01 | 1.16 |

## RESISTANCE RELAXATION TESTS

The compositions of Examples 7-15 were tested by 20 the following tests. Samples 1 inch 82.54 cm) by 1.5 inch (3.8 cm) were cut from the molded slabs. Electrodes were formed on each sample by painting a strip 0.25 inch (0.62 cm) wide at each end with a suspension of silver particles (Electrodag 504 available from Acheson 25 Colloids). The samples were annealed for 5 minutes at 200° C., and then cooled. The samples were then placed in an oven at 100° C. and their resistances measured at intervals. It was found at the lower the head-to-head content of the polymer, the less its change in resistance. 30

We claim:

1. A conductive polymer composition which comprises carbon black dispersed in a polymeric component which consists essentially of 65 to 100% by weight of a crystalline polyvinylidene fluoride which has a head-to-head content of less than 5.0%, and 0 to 35% by weight of at least one elastomeric polymer. 35
2. A composition according to claim 1 wherein the polyvinylidene fluoride has a head-to-head content of less than 4.5%.
3. A composition according to claim 2 wherein the polyvinylidene fluoride has a head-to-head content of less than 4.0%.
4. A composition according to claim 1 which contains an amount of carbon black such that the composition exhibits PTC behavior. 45
5. A device which comprises
  - (i) a conductive polymer element comprising carbon black dispersed in a polymeric component which consists essentially of 65 to 100% by weight of a crystalline polyvinylidene fluoride which has a head-to-head content of less than 5%, and 0 to 35% by weight of at least one elastomeric polymer; and

(ii) at least one electrode which is in electrical contact with the conductive polymer element.

6. A device according to claim 5 wherein the polyvinylidene fluoride has a head-to-head content of less than 4.5%.

7. A device according to claim 6 wherein the polyvinylidene fluoride has a head-to-head content of less than 4.0%.

8. A device according to claim 5 which is a self-regulating heater in which the conductive polymer composition comprises an amount of carbon black such that the composition exhibits PTC behavior.

9. A device according to claim 6 which comprises at least two electrodes which can be connected to a source of electrical power to cause current to flow through the conductive polymer element.

10. A device according to claim 6 wherein the polyvinylidene fluoride is a homopolymer of vinylidene fluoride.

11. A device according to claim 6 which contains 16 to 25% by weight of carbon black.

12. A composition according to claim 1 where the polyvinylidene fluoride is a homopolymer of vinylidene fluoride.

13. A composition according to claim 1 wherein the polyvinylidene fluoride is a copolymer of vinylidene fluoride and a comonomer which is present in amount up to 15% by weight and which is selected from tetrafluoroethylene, hexafluoropropylene and ethylene.

14. A composition according to claim 1 in which the polymeric ingredients consist essentially of the polyvinylidene fluoride and 0 to 20% by weight of at least one elastomeric polymer.

15. A composition according to claim 1 which contains 16 to 25% by weight of carbon black.

16. A composition according to claim 1 which has been cross-linked.

\* \* \* \* \*

UNITED STATES PATENT AND TRADEMARK OFFICE

**CERTIFICATE OF CORRECTION**

PATENT NO. : 4,935,156

DATED : June 19, 1990

INVENTOR(S) : Peter H. van Konynenburg et al

It is certified that error appears in the above-identified patent and that said Letters Patent is hereby corrected as shown below:

Column 7, line 21 Replace "inch82.54 cm)" by --inch (2.54 cm)---.

Claim 5, line 1 Replace "A" by --An electrical--.

**Signed and Sealed this  
Nineteenth Day of November, 1991**

*Attest:*

HARRY F. MANBECK, JR.

*Attesting Officer*

*Commissioner of Patents and Trademarks*